

Aug. 7, 1934.

K. H. TALBOT

1,969,283

PROCESS OF COATING ROAD AGGREGATES

Filed Nov. 28, 1931

2 Sheets-Sheet 1



FIG. 1

Inventor  
KENNETH H. TALBOT.

By *Rubber Coat*  
Attorneys

Aug. 7, 1934.

K. H. TALBOT

1,969,283

PROCESS OF COATING ROAD AGGREGATES

Filed Nov. 28, 1931

2 Sheets-Sheet 2



FIG. 4.



FIG. 2.



FIG. 3.



FIG. 5.



FIG. 6.

Inventor  
KENNETH H. TALBOT.

By

Ross Ross

Attorneys

## UNITED STATES PATENT OFFICE

1,969,283

## PROCESS OF COATING ROAD AGGREGATES

Kenneth H. Talbot, Milwaukee, Wis., assignor to  
National Equipment Corporation, Milwaukee,  
Wis., a corporation of Delaware

Application November 28, 1931, Serial No. 577,824

17 Claims. (Cl. 106—31)

This invention appertains to the art of preparing road aggregates such as used for the purpose of constructing secondary roads, and primary or other types of roads.

5 This invention involves a novel process for the purpose of coating mineral aggregates, such as gravel or the like, used in road construction such as referred to.

The primary aim of the invention has been 10 to devise a process of thoroughly coating each individual particle or element of the mineral, or rock, or other aggregate, that constitutes the body of the road to be made, and in the carrying out of the invention a method comprising new steps of 15 coating procedure have been evolved. The method hereof in its broader phase includes the subjecting of the mass of solid aggregates, as for instance gravel, sand, or the like, to centrifugal force, the forming of a continuously revolving or 20 moving tube of such aggregates by the application of said force, and directing against the individual constituents or particles of the moving aggregates the fluid coating which is to constitute a binder for the aggregates when laid upon the sub-grade 25 to make the road.

In accordance with the invention it is preferred to apply the coating mixture to the aggregate materials by spraying these in the form of an effective blast spray from within the tube of moving materials. In other words, the spray of the coating mixture is applied to the particles of the aggregate materials as the latter are rotated around the spray incident to the application to the materials of a centrifugal force, previously 35 referred to.

The process of this invention involves subsidiary features of the method utilized including the deflecting of the movement of the aggregates under the influence of their centrifugal force acting thereon to bring the aggregates more fully into the range of movement of the spray of coating mixture, provision for checking the volume or amount of aggregates that are being subjected to the action of the coating mixture, and provision for varying the speed of movement of the coated aggregates obtained in the practice of the process, from the point at which they are coated to the point of discharge thereof from which they are taken to the site at which they are to be laid 50 upon the road.

With the foregoing and other objects in view that will be made clear upon reviewing the following description in conjunction with the accompanying drawings, it is noted that in the drawings there is illustrated a type of machine adapted to be used for the purposes of the process of this invention. But it is not desired to be restricted to this particular type of machine by which to carry out the invention, since various 55 machines may be availed of for the purposes of

the process or method hereinafter set forth in detail.

In the accompanying drawings,

Fig. 1 is a side elevation of a machine suitable for the purpose of practicing the method of the 65 invention;

Fig. 2 is a diagrammatic view charting certain of the various mechanical parts and controlling features of a machine suitable for carrying out the process to be described;

Fig. 3 is a cross-sectional view of the drum of the coating machine illustrating generally the mode of supporting the same;

Fig. 4 is a fragmentary longitudinal sectional view of the parts generally illustrated in Fig. 3; 75

Fig. 5 is a cross-sectional view of the coating drum or barrel, illustrating the mounting of the adjustable scraper coating with the inner surface of the drum more clearly;

Fig. 6 is a view of a somewhat diagrammatic nature showing the manner in which the drum rotates and imparts to the flowing aggregates a centrifugal force that causes these aggregates to be conducted in an approximately elliptical path of movement forming them into a tube, so to 80 speak, as previously generally mentioned. The view is taken from the charge end.

The machine for carrying out the process hereof will be briefly described only, because it represents merely a preferred means by which to 90 practice the invented method and other instrumentalities of a nature to function equivalently may be restored to, if desired, for the same purposes.

In the drawings, and referring especially to 95 Fig. 1, 1 denotes a hopper adapted to contain aggregates such as used for the making of secondary or other roads. At the bottom of the hopper will be provided a gate or valve, not clearly shown, but operable manually to supply the 100 aggregates within the hopper to a suitable conveyor 2 of the belt type. The conveyor 2 is pivotally supported at one end, as at 3, whilst its opposite or right hand end is carried by a flexible member 4 of a weighing indicator 5. The purpose 105 of the indicator 5, which does not form a part of this invention as presented in this application, is to enable the operation of the machine in such a manner as to supply a uniform or predetermined quantity of materials passing from the 110 hopper 1 by means of the conveyor 2, to the coating drum 6 of the machine. From the conveyor 2 the aggregate materials pass to a feeding chute 7 rotatively mounted so that its lower end may enter the upper end of the drum 6 or may be 115 turned into a position to supply materials to a container or place other than the drum 6. The coating mixture is carried in a large storage tank 8 within the framework of the machine, said tank 120 communicating with the pump line by means of

a conduit 10 leading to the tank 8, in which conduit is located the strainer 11. From the pump 9 the coating mixture is forced through the pipe 12 to the pipe 13 and at the juncture of the pipes 12 and 13 is located a regulating valve 14. Connected with the pipe 13 is a swinging nozzle 15 movable into the upper end of the drum 6, and swingable to the outer position illustrated in Fig. 1 when it is desired to check the volume of flow 10 of the coating mixture from said nozzle. Joining with the pipe 12 is a by-pass pipe or conduit 16 which leads back to the tank 8, and in the length of this conduit 16 is a pressure release valve 17. The upper portion of the drum 6 is 15 carried by trunnions 18 and the lower portion is supported by trunnion members 19 connected with lifting yokes 20 operable by actuating screws 21 having hand wheels 22. By manipulation of the parts 19 to 22 the lower end of the drum 6 20 may be raised and lowered to vary the velocity of movement of the coated aggregates passing through the drum.

Referring to Figs. 3 to 6 inclusive, it is noted that within the drum 6 at its upper portion is 25 mounted a scraper 23 adjustably carried by screw means 24 so that the scraping edge 23a thereof may be moved and held in proper relation to the inner wall or surface of the drum 6 for purposes to be hereafter described. In the drum 6 30 as seen in Fig. 6 is the spray nozzle 15, previously referred to.

With an understanding of the machine for practicing the purposes hereof, as given above, the cycle of operation incident to the method of 35 this invention will now be set forth. The aggregate materials from the hopper 1 pass to the conveyor 2, are supplied to the feed chute 7, and enter the drum 6 at its upper end portion. The aggregate materials are preferably dry when they 40 enter the drum and are to be coated with a coating mixture of a bituminous or other suitable nature, as they are operated upon within the drum. When the aggregate materials enter the drum the latter is in motion, being rotated at a comparatively 45 high velocity, say approximately 60 R. P. M. for a drum of approximately 24" diameter, and in this way motion is imparted to the mass of the aggregate materials. The centrifugal force obtained from the rotating moving drum 6 is imparted to the aggregate materials as they enter 50 the upper end of the drum, the materials being thus lifted by traveling of the drum in its direction of rotation and being engaged near the top portion of the drum by the scraper 23. The 55 scraper 23 disengages the materials from the inner wall of the drum and directs them downwardly with a deflecting function somewhat after the manner depicted in Fig. 6, both the aggregate materials operated on in the manner described having motion imparted thereto, giving 60 to them a substantially tubular form. That is, the aggregate materials move in a circular path, creating the form of a tube of such materials so that there is a space surrounded by the path of 65 their movement. In this tube, or in the space within the moving of aggregate materials, is located the spray nozzle 15 from which, under high pressure, the coating mixture is sprayed against the moving materials surrounding the same and 70 acted on by the drum. In this way the aggregate materials are coated with great thoroughness and the operation of supplying the materials, coating the same and discharging them takes place continuously in a very effective manner.

Referring to the diagram illustration of Fig. 2, the control of the process may become readily apparent. The coating mixture is seen issuing from the nozzle 15 of the pipe line 13. The pressure regulating valve 14 may be opened or closed to control the volume of oil used per unit of time. The bypass valve 17 may be opened or closed to bypass back to the tank a greater or less quantity of the coating or bituminous mixture. The pump 9 is a constant speed pump and the use of the valve 17 enables variation in the pressure at the nozzle 15. The burner 25 may be utilized for heating the coating mixture for obvious purposes.

It is notable that the scraping appliance 23 performs a separate function independently of its scraping action relative to the drum 6. It acts to deflect the direction of movement of the mass of materials from the path they would ordinarily take due to the effect of the centrifugal force thereon, as illustrated in Fig. 6, so as to impart to the particles or individual elements of the materials a special agitation tending to break or separate the particles, and move them independently of the other movement which has been described. In other words, this action might be characterized as a special agitation imparted to the materials that greatly increases the efficiency of the machine insofar as the proper coating of the particles of the mass is concerned.

As stated above, the centrifugal force primarily imparts to the mass its tubular form in the nature of a deflective tubular shaft of rotating or moving particles and since the spray nozzle supplies the coating mixture under pressure at the point described the coating substance is caused to penetrate the materials by entering the interstices between the particles in such a manner that all the particles are coated effectively over the whole superficial area thereof. Where the mass of materials is of a finer nature, such as sand or the like, it is evident that the employment of the scraping and agitating means 23 is especially important. Therefore, it is clear from the foregoing that the materials of the aggregate are caused to move in a defined orbit and whilst they are moving in such orbit there is imparted to the particles of these materials movement relative to each other and during these movements of the particles they are thoroughly coated.

It is to be borne in mind that the process of this invention is susceptible of use for coating aggregates or minerals, or fine particles of materials of any sort, the process of the invention not being confined obviously to the use thereof in the art of preparation of aggregates for road purposes alone. It is notable also that in the practice of the invention, the materials are maintained in their tubular shape so to speak, as they are raised from the bottom of the drum and travel up to the point where they strike the member 23. At this point there is a scattering action so that a portion of the materials may actually be thrown downwardly and outwardly to strike the drum at a point at the bottom of its periphery, while other materials because of their movement within the mass as the material strikes the cut off or scraper blade 23, are thrown downwardly and inwardly so that they strike the periphery of the drum above the lowest point of the path of movement. In other words, the effect of the blade or scraper member 23 is to deflect the shape of the tubular form imparted to the mass by the centrifugal force incident to the movement of the drum.

- The method of moving the materials as above described is important and makes for the uniformity of coating so desirable as a result of the practice of my process. Moreover, the manner of scattering the materials to a certain extent in their centrifugal movement affords very effective results as regards the action of the spray of the coating material because said spray is thus enabled to coat the surface of the individual particles of the materials. Following the action of spraying incident to my process, there is the additional action of rubbing of particle on particle thus distributing the fluid coating by so doing.
- Having thus described my invention, what I claims as new and desire to secure by Letters Patent of the United States is:
1. The method of treating road aggregate materials which comprises imparting to the materials motion forming them into a moving tubular mass, and coating the materials with a coating substance applied to such moving mass and particles thereof.
  2. The method of treating road aggregate materials which comprises imparting to the materials motion forming them into a moving tubular mass, spraying a coating mixture upon the mass as it moves, and causing advancing of the mass in the direction of its axis.
  3. The method of treating road aggregate materials which comprises imparting to the materials motion forming them into a moving tubular mass, and applying a coating mixture to the mass from a point surrounded by the moving materials thereof.
  4. The method of treating road aggregate materials which comprises imparting to the materials motion forming them into a moving tubular mass, and applying a coating mixture to the mass from a point surrounded by the moving materials thereof while advancing the mass in the direction of its axis of movement.
  5. The method of treating road aggregate materials which comprises subjecting the materials to centrifugal force to cause them to assume the condition of a tubular shaft of moving aggregate particles, and coating them while so moving.
  6. The method of treating road aggregate materials which comprises subjecting the materials to centrifugal force to cause them to assume the condition of a tubular shaft of moving aggregate particles, and spraying such particles with a coating mixture from a point within the space surrounded by the materials.
  7. The method of treating road aggregate materials which comprises subjecting the materials to centrifugal force to cause them to assume the condition of a tubular shaft of moving aggregate particles, spraying such particles with a coating mixture from a point within the space surrounded by the materials, and causing the mass of materials to shift lengthwise of its axis of movement during the spraying operation.
  8. The method of treating road aggregate materials which comprises imparting to the materials motion forming them into a moving tubular mass, causing motion of each particle of the materials relative to adjacent particles, and coating the materials with a coating substance applied to such moving mass and particles thereof.
  9. The method of treating road aggregate materials which comprises imparting to the materials motion forming them into a moving tubular mass, applying friction to certain particles of the mass to impart movement thereto and create movement of those adjacent particles contacting therewith, and coating the materials with a coating substance applied to such moving mass and particles thereof.
  10. The method of treating road aggregate materials which comprises subjecting the materials to centrifugal force causing said materials to assume and form a hollow moving mass, and applying to the materials a coating substance while so moving.
  11. The method of treating road aggregate materials which comprises subjecting the materials to centrifugal force causing said materials to assume and form a hollow moving mass, causing agitation of the materials separate from their movement by the centrifugal force, and applying to the materials a coating substance while so moving.
  12. The method of treating road aggregate materials which comprises imparting to the materials motion forming them into a moving tubular mass, agitating the particles of the moving tubular mass, and coating the materials with a coating substance applied to such moving mass and particles thereof.
  13. The method of treating road aggregate materials which comprises imparting to the materials motion forming them into a moving tubular mass, applying a coating mixture to the mass from a point surrounded by the moving materials thereof, and agitating the particles of the mass additional to their movement in their tubular arrangement.
  14. The method of treating road aggregate materials which comprises imparting to the materials motion in a defined closed orbit, subjecting the materials at such time to such movement as to cause motion of the particles thereof relatively to each other, and coating the particles of the materials whilst being subjected to the said movement.
  15. The method of treating road aggregate materials which comprises imparting to the materials motion in a defined closed orbit, subjecting the materials at such time to such movement as to cause motion of the particles thereof relatively to each other, and coating the particles of the materials whilst being subjected to the said movement with a coating mixture under pressure causing entrance thereof into the interstices between all particles of materials.
  16. The method of treating road aggregate materials which comprises imparting to the materials motion forming them into a moving tubular mass, and applying a coating mixture to the mass from a point surrounded by the moving materials thereof with a positive pressure force acting upon the coating mixture.
  17. The method of treating road aggregate materials which comprises subjecting the materials to centrifugal force causing said materials to assume and form a hollow moving mass, causing agitation of the materials separate from their movement by the centrifugal force, applying to the materials a coating substance while so moving, and causing the coating substance to be applied under pressure.

KENNETH H. TALBOT.